# EUROPEAN PATENT SPECIFICATION

(11) **EP 0 179 527 B1**
(45) Date of publication and mention of the grant of the patent: **03.06.1992**
(21) Application number: 85201675.7
(22) Date of filing: 11.10.1985
(51) Int. Cl.: H01B 3/10, B21C 37/04

(54) **Sheathed reinforcing wire**
Ummantelter Verstärkungsdraht
Fil de renforcement gainé

(30) Priority: 18.10.1984 NL 8403188
(43) Date of publication of application: 30.04.1986
(73) Proprietor: Koninklijke Schelde Groep B.V., NL-4381 SE Vlissingen (NL)
(72) Inventor: van der Goes, Jacobus Johannes, NL-4386 AS West-Souburg (NL)
(74) Representative: van der Beek, George Frans, Ir.

(56) References cited:
- EP-A- 0 003 370
- EP-A- 0 015 621
- DE-B- 1 298 680
- DE-B- 2 454 620
- GB-A- 983 023
- US-A- 3 109 053
- US-A- 3 222 219

## Description

The invention relates to a structure which in view of its working conditions, such as temperature and medium, consists of certain materials, but which materials have a per se inadequate strength and/or dimensional stability at high working temperature.

Examples of structures of this type are pipes and containers for the process industry and nuclear energy, but also moulds, in particular extrusion moulds.

In the said pipes and containers very aggressive media and high temperatures and pressures are often used. In view of this pipes and containers of this type are often constructed of nickel or a nickel-based alloy or of other heat- and medium-resistant materials. At very high temperatures, however, many of these materials lose their strength and dimensional stability. Problems of this type may occur, for example, in extrusion moulds in which very high pressures are generated and through which flows the material to be extruded. Therefore for these structures temperature and pressure limits exist which are determined by the material of the structures, as a result of which their application is subject to limitations, whereas they could, in view of the properties of, for example, nickel or nickel alloy, withstand much higher temperatures and more aggressive media. This means that structures of this type cannot be ideally utilized, even if the material is extremely suitable for certain working conditions.

A pipe structure consisting of a nickel alloy is already known which, as a result of the use of a reinforcing wire of molybdenum, can work at much higher internal pressure and higher temperature than without the reinforcing wire, as a result of which the efficiency of the process in the pipe is considerably increased. By using the said reinforcing wire the temperature can be increased from 900°C to 1,300°C and the pressure from 200 to 300 kpa.

It has emerged, however, that under certain circumstances the molybdenum of the reinforcing wire is attacked, as a result of which its strength decreases. At high temperature molybdenum will, for example in the presence of oxygen, oxidise to volatile molybdenum trioxide, as a result of which it becomes brittle and vaporises. At these high temperatures molybdenum may in addition diffuse into the material of the structure in which it is incorporated as a reinforcing wire and with which it is in close contact. Oxygen residues which may still be present locally after manufacture may again result in molybdenum trioxide. The molybdenum may in addition form metallic compounds which have completely different properties with the material of the surrounding structure. The material of this structure may also diffuse into the molybdenum.

The abovenamed unfavourable factors may be present separately, but also in combination, as a result of which their degenerative influence on the reinforcing wire in general increases considerably as the metal temperatures rise. The above limits the use of the reinforcing wire art consequently the use of the said beneficial materials for the pipes, containers and moulds, etc.

The abovenamed drawbacks are now eliminated in a structure of the present invention which is characterized in that this structure is reinforced by a sheathed reinforcing wire which is successively built up coaxially from a core wire, which provides the reinforcement, a barrier layer of ceramic and a thin metal sheath.

The ceramic may possess the form of a powder in an extremely compressed state, but it can also be applied by means of per se known physical or chemical vapour deposition processes, in which case the said coating will possess in general a crystalline structure, as a result of which an adequate density is also obtained, which in the case of a coating may approach 100%. A vapour deposited coating of this type must have a minimum thickness of approx. 10 µm. In the case of moulded ceramic powder the density will in general be in the range of 60 to 80%.

The present invention also provides a sheathed reinforcing wire characterized in that the wire is successively built up coaxially from a core wire consisting of molybdenum, tantalum or niobium or of other materials with high heat resistance and a low coefficient of expansion, but with the drawback that they readily oxidize, diffuse and vaporize at high working temperatures, while they do not of themselves form any protective oxide skin.

The sheathed reinforcing wire according to the invention is protected against these disadvantageous effects by the barrier layer of ceramic so that it is not sensitive or is sensitive to a much lesser extent to the abovenamed negative influencing factors.

The ceramic powder, which may in particular consist of Al₂O₃, SiC, Si₃N₄ or MoSi₂ or mixtures thereof, may be applied to the core wire in diverse manners.

DE-B-2,454,620 discloses a process of making a sheathed wire built up coaxially from a core wire, a ceramic barrier layer and a metal sheath. However, this does not relate to a reinforcing wire, but instead to a method for making a thermo-element preform, consisting of coaxial elements. This thermo-element preform cannot be used as reinforcing wire, because the core wire has no reinforcing function and therefore will not be made of particularly resistant material in connection with this function. The only consideration for the choice of this core wire material is the function as a thermo-element and having the most suitable electrical resistance. Also the material combination for the core wire and the exterior sheath wire will be concentrated on the thermo-electric function and such materials are very well known and are not the materials for the reinforcement wire. The characteristics and thickness of the ceramic intermediate layer in a thermo-element are chosen exclusively in connection with electrical insulation. In a reinforcement wire the ceramic intermediate layer serves to prevent diffusion between the core wire material and the sheath material and also as a matter of course, between the ceramic layer itself and the core and sheath. This intermediate layer could be even electrically conducting, which in a thermo-element certainly cannot be accepted.

The density of the ceramic layer in a reinforcing wire is much more relevant than in a thermo-element wire. This density is of importance for the entrapped gas, such as oxigen, and the axial movement of the gas (diffusion), which would affect the life of the reinforcement function of the wire. The essence of DE-B-2,454,620 is the thermo-coax element itself, in which this thermo-element is formed by a core wire and a sheath, electrically insulated by a ceramic intermediate layer. Generally known thermo wires consist of two core wires, but made in the same way as in DE-B-2,454,620, and in which the sheath serves to keep these two wires together. This inventive idea herein is so different from the use as reinforcing wire as in the present invention, that there cannot be any suggestion to use the thermo-element preform as reinforcing element.

In one manufacturing process a flat strip of the sheath material, for example consisting of a nickel-based alloy such as inconel, is bent into a tube closed along a seam around the core wire in a continuous drawing process, such as is known in the manufacture of electrical wires and cables, by means of a former. Immediately before the bending into a tube, the ceramic powder is fed onto the metallic strip in a quantity such that, when the strip is bent into a tube, the ceramic powder is firmly pressed together and compressed. The seam of this closed tube is then sealed by welding, for example by means of a laser beam. After this the reinforcing wire thus formed can be reduced in diameter by means of further drawing processes, as a result of which the ceramic powder is compressed still further.

The quantity and compression of the ceramic powder depends on the expected working conditions in which the reinforcing wire will be used. The thickness and also the compression of the ceramic powder must be such that no oxygen can penetrate to the core wire and the material of the core wire cannot diffuse to the outside, while material from the surrounding structure can also not reach the core wire by diffusion. The ceramic powder must, in addition, have a high degree of purity, in particular there must be no materials present therein such as metals with which the metal of the core wire may form harmful compounds or metallic elements which may diffuse into the core wire. The thickness of the protective ceramic layer is also determined by the additionally necessary bends which the wire must be able to undergo when applied as reinforcing wire in or on a structure to be reinforced.

In another manufacturing process a relatively thick, short reinforcing wire with ceramic powder applied around it and an outer sheath in the form of a coaxial cylinder with a likewise relatively large diameter is subjected to a drawing process in which the assembly thus obtained in successively fed through drawing dies with increasingly smaller diameter until the assembly finally has the desired outer diameter. In this drawing process the ceramic powder will also be considerably compressed.

The above manufacturing methods can of course also be used if the ceramic is applied by means of.the physical and chemical vapour deposition processes mentioned. The coating thus obtained will in general have a crystalline structure, which guarantees a good sealing of the parts with respect to each other.

The reinforcing wires according to the invention may be embedded in the structure to be reinforced, but they may also be applied, for example, on the outside around a pipe or container or mould, for example wound, woven or braided. The distances between the mutual reinforcing wires in this woven structure or braiding work depend of course on the desired strength of the structure. As a result of the protective layer of the reinforcing wire these reinforcements can now also be applied on the side of the structure in which the media occur which would have a very aggressive action on the bare reinforcing wire.

If the reinforcing wire is embedded, the space between the wound or braided wires will preferably be filled up with suitable metal powder, for example nickel powder with a grain size less than 50 µm which is compressed under pressure to 60% or more. (A density of 100% corresponds to the specific gravity of the pure metal.) If the reinforcing wire is embedded, consideration can also be given to a structure in which the said wires are applied to the outside, for example wound as mentioned above, and in which a thin metal sheath is moulded around the said wires which does not per se contribute to the strength of the structure. In this case the space between the separate sheathed reinforcing wires will also preferably be filled with the said metal powder.

The thickness of the core wire of the reinforcing wire according to the invention depends on the stress to be taken up by the said wire, i.e. on the degree to which the structure must be reinforced. The wire may of course be thinner if the braiding work is closer.

A test wire according to the invention which was sucessfully tested had a total final thickness of 3 mm. The core wire had a thickness of 1.2 mm, while the seam-welded outer sheath was 0.3 mm thick. These dimensions were achieved after a drawing process. For this purpose the sheathed reinforcing wire had a thickness of 3.2 mm after the bending of a metal strip around the core wire in the manner previously described and the sealing of the seam by welding. With this thickness the ceramic powder was already so compressed that it could not fall loosely out of the space between the core wire and the sheath.

It is self evident that the invention is not limited to the special reinforcing wires described above but that modifications and amplifications are possible without going beyond the scope of the invention. The cross-section of reinforcing wire will in general be round, but it may also be elliptical. The same applies of course to the core wire. The reinforcing wires according to the invention can be manufactured to any desired length and applied in or on the structures to be reinforced.

## Claims

1. A structure having per se an inadequate strength and/or dimensional stability at high temperature, characterized in that this structure is reinforced by a sheathed reinforcing wire, which is successively built up coaxially from a core wire, which provides the reinforcement, a barrier layer of ceramic and a thin metal sheath.

2. Reinforcing wire, characterized in that the wire is successively built up coaxially from a core wire consisting of molybdenum, tantalum, or niobium, a barrier layer of ceramic and a thin metal sheath.

3. Wire of claim 2, characterized in that the ceramic consists of a powder in an extremely compressed state.

4. Wire of claim 2, characterized in that the ceramic consists of a coating with an in general crystalline structure which is deposited on the core wire by means of physical vapour deposition processes (PVD) or chemical vapour deposition processes (CVD).

5. Wire of claims 2, 3 and 4, characterized in that the ceramic powder consists of Al₂O₃, SiC, Si₃N₄ or MoSi₂ of adequate purity or mixture thereof.

6. Wire of claims 2-5, characterized in that the thin metal sheath consists of nickel or a nickel-based alloy.

7. Wire of claim 6, characterized in that the thin metal sheath consists of a metal strip bent into a tube and seam-welded.

8. Use of a wire as claimed in claims 2-7, as a reinforcing wire for structures which have inadequate strength and/or dimensional stability at high temperatures.

## Revendications

1. Structure présentant en soi une solidité et/ou une stabilité de dimensions insuffisantes à haute température, structure caractérisée en ce qu'elle est renforcée par un fil de renforcement gainé constitué successivement et coaxialement d'un fil formant noyau assurant le renforcement, d'une couche formant barrière en céramique et d'une gaine métallique mince.

2. Fil de renforcement caractérisé en ce qu'il est constitué successivement et coaxialement d'un fil formant noyau en molybdène, en tantale ou en niobium, d'une couche formant barrière en céramique et d'une gaine métallique mince.

3. Fil selon la revendication 2, caractérisé en ce que la céramique est constituée d'une poudre dans un état extrêmement comprimé.

4. Fil selon la revendication 2, caractérisé en ce que la céramique est constituée d'un revêtement à structure en général cristalline déposé sur le fil formant noyau par un processus de dépôt à la vapeur physique (PVD) ou par un processus de dépôt à la vapeur chimique (CVD).

5. Fil selon l'une quelconque des revendications 2 à 4, caractérisé en ce que la poudre de céramique est constituée de Al₂O₃, de SiC, de Si₃N₄ ou de MoSi₂ présentant une pureté convenable, ou de mélanges de ces éléments.

6. Fil selon l'une quelconque des revendications 2 à 5, caractérisé en ce que la gaine métallique mince est constituée de nickel ou d'un alliage à base de nickel.

7. Fil selon la revendication 6, caractérisé en ce que la gaine métallique mince est constituée par une bande de métal mince courbée en forme de tube et dont le joint est soudé.

8. Utilisation d'un fil selon l'une quelconque des revendications 2 à 7, comme fil de renforcement pour des structures présentant une solidité et/ou une stabilité de dimensions insuffisantes à températures élevées.

## Patentansprüche

1. Gebilde, welches an sich eine unzulängliche Festigkeit und/oder Dimensionsstabilität bei hoher Temperatur hat, dadurch gekennzeichnet, dass dieses Gebilde durch einen ummantelten Verstärkungsdraht verstärkt ist, welcher sukzessiv koaxial aufgebaut wird, aus einem Kerndraht welcher die Verstärkung bildet, einer Sperrschicht aus Keramik und einer dünnen Metallummantelung.

2. Verstärkungsdraht, dadurch gekennzeichnet, dass der Draht sukzessiv koaxial aufgebaut wird, aus einem Kerndraht welcher aus Molybden, Tantal oder Niob besteht, einer Sperrschicht aus Keramik und einer dünnen Metallummantelung.

3. Draht nach Anspruch 2, dadurch gekennzeichnet, dass das keramische Material ein Pulver in einem extrem komprimierten Zustand ist.

4. Draht nach Anspruch 2, dadurch gekennzeichnet, dass das keramische Material aus einem Überzug mit einer im allgemeinen kristallinen Struktur besteht, welche auf dem Kerndraht mit Hilfe physikalischer Aufdampfverfahren (PVD) oder chemischer Aufdampfverfahren (CVD) aufgebracht ist.

5. Draht nach Anspruch 2, 3 und 4, dadurch gekennzeichnet, dass das Keramikpulver aus Al₂O₃, SiC, Si₃N₄ oder MoSi₂ mit entsprechender Reinheit oder Gemischen hiervon besteht.

6. Draht nach den Ansprüchen 2 bis 5, dadurch gekennzeichnet, dass die dünne Metallummantelung aus Nickel oder einer Legierung auf Nickelbasis besteht.

7. Draht nach Anspruch 6, dadurch gekennzeichnet, dass die dünne Metallummantelung aus einem Metallband besteht, welches zu einem Rohr gebogen und nahtgeschweisst ist.

8. Verwendung eines Drahtes nach den Ansprüchen 2 bis 7 als ein Verstärkungsdraht für Gebilde, welche eine unzulängliche Festigkeit und/oder Dimensionsstabilität bei hohen Temperaturen haben.
